

## UNITED STATES PATENT OFFICE

2,137,782

## LUBRICATING COMPOSITION

Carl F. Prutton, Cleveland, and Albert K. Smith, Shaker Heights, Ohio, assignors, by mesne assignments, to The Lubri-Zol Development Corporation, Cleveland, Ohio, a corporation of Delaware

No Drawing. Application July 16, 1935,  
Serial No. 31,720

18 Claims. (Cl. 87—9)

In U. S. Patent Nos. 1,986,645 and 1,986,651 it is taught that the lubricating properties of a lubricating composition may be materially improved and extreme pressure characteristics imparted to lubricants such as mineral lubricating oil, by the addition thereto of minor amounts of halogenated carbon ring compounds.

It has been explained that the reason why such compounds thus improve the extreme pressure characteristics of the lubricant probably is due to the fact that such addition agents chemically react with the bearing surfaces under the conditions imposed by relative movement and extreme pressure between the bearing surfaces to form a microscopic film of a metallic halide which prevents seizing between the bearing surfaces by acting as an anti-fluxing agent.

The halogenated carbon ring compounds were indicated as preferable in said patents due to the fact that such compounds are relatively stable, i. e., they do not readily hydrolyze in the presence of moisture which usually occurs in varying quantities in mineral oils. In other words, the halogenated carbon ring compounds are sufficiently stable so that decomposition and attack thereof upon the metallic surfaces occurs only in the areas where extreme pressure is encountered, i. e., on the bearing surfaces.

One theory of the action of halogen compounds, specifically chlorine compounds, in increasing film strength, assumes that, as above indicated, under the stress of the rubbing action of bearing surfaces in motion under load, chlorides of the bearing metals are formed on their surfaces and exert an anti-fluxing effect in preventing subsequent fusing of the two surfaces. This surface reaction, however, to take place with sufficient effectiveness depends upon the hydrolysis of the chlorine compound as a simultaneous intermediate reaction. These reactions may be expressed as follows:



where R is an organic radicle and M is one of the metals of the bearing surfaces.

(NOTE:—The hydrogen evolved by (2) probably would act to reduce one or more of the organic compounds rather than to appear as free hydrogen.)

The correctness of the foregoing theory is substantiated by the fact that when a chlorinated hydrocarbon is added to a hydrocarbon mineral oil and the mixture thoroughly freed from moisture, by the action of dehydrating agents, the film strength is no more than that of the oil alone. Exposure of the mixture to the atmosphere so that it may absorb a slight amount of moisture will then cause an increase in the film strength.

Since the presence of a large amount of moisture and especially of free water is objectionable in a lubricant besides being a highly variable factor in normal service, it is advisable to supply an oil soluble substitute for the same.

It is the principal object of this invention, therefore, to provide a lubricating composition of the type utilizing halogenated organic compounds as the extreme pressure addition agent but so modified as to be effective in the manner defined without being dependent upon the presence in the lubricating composition of some addition material such as water.

Other objects of our invention will appear as the description proceeds.

To the accomplishment of the foregoing and related ends, said invention, then consists of the means hereinafter fully described and particularly pointed out in the claims.

The following description sets forth in detail one approved combination of ingredients embodying our invention, such disclosed means constituting, however, but one of various forms in which the principle of the invention may be used.

Broadly stated, this invention comprises the use as a lubricant of oxygen and halogen bearing organic compounds and more specifically, oxygen and halogen bearing organic ring compounds, either used alone or incorporated with any suitable oil base.

The oxygen which is included in the molecule of the addition agent acts to increase the effectiveness of the latter in raising the film strength of a mineral oil to which the addition agent is added or to improve the lubricating properties of the halogenated compound when used without the addition of some other lubricant. The oxygen probably acts in the same way as water in making possible the formation of hydrochloric

acid as an intermediate step in the surface reaction above explained.

By combining in a single molecule the halogen and the oxygen atoms, a lubricant is affected in two ways:—

First: The oxygen is always available at the exact point where required; and

Second: The molecule is more strongly adsorbed by metal surfaces than similar halogen compounds which do not contain oxygen.

The latter circumstance enhances the effect of small amounts of such compounds because it is equivalent to an increase in concentration of the compound at the bearing surfaces.

15 We have found that certain oxygen-containing organic ring compounds which have been chlorinated and added to a lubricating oil are capable of improving the properties of such oil, particularly when employed for "thin-film" lubricating purposes. The addition of these certain oxygen containing organic ring compounds which have been chlorinated and added to the lubricating oil have been found to improve the properties thereof to an even greater extent than certain similar chlorinated hydro-carbons, notably when added in very small amounts.

18 The halogen and oxygen-containing organic ring compounds added to a suitable oil base are, as above indicated, preferably of the chlorinated species and particularly the compounds which have been found to produce very satisfactory results, may be classified as follows; viz:

*I. "Carbon ring" type compounds*

35 (a) Of the aromatic, or allied type, including oxygen and halogen bearing derivatives of benzene, diphenyl, naphthalene, anthracene, etc., and homologs of them, also such derivatives of compounds of the bridged ring type, such as the terpenes, and related compounds.

40 (b) Of the class including such derivatives of the cyclo-aliphatic compounds such as cycloparaffins, cyclo-olefines, cyclo-acetylenes. Examples of this class are oxygen and halogen-bearing derivatives of hydrogenated aromatic compounds, such as the following:

45 (1) Hydrogenation products of benzene (e. g. cyclohexane, cyclohexene, cyclohexadiene).

(2) Hydrogenation products of naphthalene (e. g. decahydronaphthalene, tetrahydronaphthalene etc.).

50 (3) Naphthenes, naphthenic acid, etc.

(c) Of mixed type such as oxygen and halogen-bearing derivatives of indene, hydrindene, hydranthracene, etc.

*II. "Heterogeneous ring" type compounds*

60 (a) Of the aromatic or allied type including oxygen and halogen-bearing derivatives of pyridine, quinoline, etc.

(b) Other types such as oxygen and halogen-bearing derivatives of furan and its derivatives and of thiophene, pyrrole etc.

Included in Class II are two principal types of compounds, viz:—Compounds in which all of the ring structures are of the heterogeneous type and compounds containing both heterogeneous ring structures and carbon ring structures.

The foregoing compounds may also be classified according to the nature of the attachment of the oxygen to the compound, viz:—

I'. Directly attached to one or more carbon atoms, as in the case of:

(1') Ethers and analogous compounds

(2') Compounds containing the  $\equiv\text{C}-\text{OH}$  5 radicle, such as alcohols and other derivatives of carbinol (including phenols, cresols, naphthols etc.)

(3') Compounds containing the carbonyl (=C=O) radicle, such as aldehydes, 10 ketones, organic acids, esters and salts of organic acids, thio-acids and esters of thio-acids

(4') Compounds in which oxygen forms a part of the ring structure, e. g. furan and its derivatives, anthraquinone, 15 etc.

II'. Indirectly attached through the means of some other atom, i. e., in the form of an inorganic radicle, e. g.: amide, arsenate, arsenite, chlorate, chlorite, cyanate, hydroxylamine, hypochlorite, nitrate, nitrite, 20 nitro, nitroso, perchlorate, phosphate, phosphite, sulphate, sulphite, sulphonic acid, sulphone, sulphuric acid, sulphoxide, thiocyanate, isothiocyanate, thio-sulphate, 25 thio-phosphate, and isocyanate.

The halogen and oxygen-bearing organic ring compounds of the ester and salt type include compounds of the aromatic type which may be classified as follows:—

1. Esters and salts of an aromatic acid;

2. Esters formed by the combination of a phenol, cresol, naphthol, etc. with an organic acid of either the fatty or aromatic type;

3. An ester formed by the combination of an 35 aromatic alcohol (either mono-hydric or poly-hydric) with an organic acid of either the fatty or aromatic type.

In addition to the substituents containing oxygen, other substituents may also be present without destroying, and in certain cases, improving the effect on the lubricating qualities of the oil such as other aryl groups, alkyl groups, and amino and substituted amino groups, imino, azo, hydrazo, hydrazine, nitrile, mercapto, sulphide, 45 polysulphide.

As a matter of convenience, the halogen and oxygen-containing substituted diphenyls, as well as the halogen and oxygen-containing substituted benzenes where two or more phenyl groups 50 are directly linked, may be inclusively referred to as halogen and oxygen-containing substituted polyphenyls.

As previously indicated, the foregoing so-called addition agents may, for most uses, be added in 55 minor amounts to other lubricants such as mineral oil, fish oil, lard oil, castor oil, rape-seed oil, etc., and in some cases, depending upon the character of use, as well as the character of the selected agents, the latter may be effectively used in their pure state.

The optimum amount of the halogen compound to be employed is usually dependent upon various considerations such as its cost, the character of the selected compound, the character 65 of the addition agent to which the same is added and more particularly, the character of the use to which the same is put. For most uses, since the cost of such halogen compounds is usually considerably greater than lubricants such as mineral oil, optimum results are obtained by using minimum quantities of these halogenated addition agents. For the purpose of lubricating and reducing the friction between relatively moving parts of an internal combustion engine such as 70

crank case bearings, piston and cylinder surfaces, as well as piston rings and valves, a composition according to our invention comprises a major proportion of a suitable oil base such as mineral oil and concentrations of from one-fourth of 1% to 2% of halogen compounds of the above defined type. If the valve structure of the engine is to be lubricated separately from the remainder of the mechanism by means acting in an auxiliary fashion such as by the addition of the lubricating composition to the engine fuel, the composition for such purposes will preferably contain a larger amount of such halogen compounds, i. e., from about 2% to about 10%.

When lubricating bearing surfaces such as gears and the like where extreme temperatures are usually not encountered a composition comprising a major proportion of a suitable oil base and a total of less than about 20% of at least one halogen and oxygen-containing organic compound of the enumerated class will be found very satisfactory.

When combined with a lubricating oil such as mineral oil, the optimum amount of the halogen compound to be employed will depend largely upon the halogen content of the particular compound, its physical characteristics and especially its effect on the viscosity of the oil to which it is added. When addition agents of the above enumerated class having very low viscosity are employed, and added to lubricants such as mineral oil, the limit of the amount of such compounds which may be added and which will produce improved results depends in a large measure upon the reduction in viscosity of the composition caused by the addition of such compounds. When, however, the more viscous compounds are employed, or where the particular use does not require thick film lubrication, the so-called addition agents may, as previously indicated, be employed in their pure state.

Experiments have shown that when compounds which readily hydrolyze, such as chlorinated open chain compounds, are added to the oily base, hydrolysis will take place to such an extent that the metal parts of any machine being lubricated will be seriously attacked and corroded by the acid generated. On the other hand, the addition of chlorinated organic ring compounds of the above enumerated class does not cause corrosion.

Certain of the halogen and oxygen-bearing open chain or aliphatic compounds, in their pure state, or when added to a suitable base do result, however, in a lubricant particularly suitable for certain purposes. Examples of the foregoing are halogenated fatty oils such as chlorinated cottonseed oil and chlorinated cocoanut oil. As above indicated, such compounds readily hydrolyze and while thus not preferred as a lubricant for use in the crank case of internal combustion engines are, nevertheless, admirably suited for use as lubricants in metal working such as drawing, extruding, rolling, etc., where the lubricant is in contact with the metallic surface for only relatively a short length of time and where the very slight amount of corrosion which may result is not particularly objectionable. Furthermore, such compounds are admirably suited for use in lubricants in die drawing or similarly working certain corrosion resistant materials such as stainless steel and the like.

With regard to the stability of the organic ring compounds contemplated, the most resistant to hydrolysis of the halogen are those in which the

halogen is directly attached to an atom which is part of a benzenoid ring structure. Examples of such ring structures are aryl groups such as the phenyl and naphthyl groups. In any case, for most uses, it is preferred to have the halogen attached to an atom which is part of an organic ring structure and especially a six-membered organic ring structure. 5

The compositions comprising our invention have certain advantages when used as a lubricant 10 of which the following may be mentioned:—

First: By the use of this composition, it is possible to extend the pressure range between the bearing surfaces because of the reduced tendency for bearing surfaces so lubricated to become 15 scored or to seize at higher pressures than are allowable with ordinary lubricants.

Second: The friction between the bearing surfaces is reduced, especially in the higher pressure range, below that obtained with ordinary lubricants. 20

This application is a continuation in part of co-pending applications Serial No. 649,734, filed December 31, 1932, and Serial No. 737,070, filed July 26, 1934. 25

Other modes of applying the principle of our invention may be employed instead of the one explained, change being made as regards the materials employed in carrying out the process, provided the ingredient or ingredients stated in any 30 of the following claims or the equivalent of such stated ingredient or ingredients be employed.

We, therefore, particularly point out and distinctly claim as our invention:—

1. A lubricating composition including as a primary lubricating constituent a halogenated oxygen-bearing organic compound in a lubricating oil vehicle, said compound having a vapor pressure less than atmospheric at a temperature of 140° C. 35

2. A lubricating composition including as a primary lubricating constituent a halogenated oxygen-bearing organic ring compound in a lubricating oil vehicle.

3. A lubricating composition including as a primary lubricating constituent a halogenated oxygen-bearing aromatic compound in a lubricating oil vehicle. 45

4. A lubricating composition containing as a principal lubricating constituent a major amount of mineral lubricating oil with the properties of such composition affecting its use as a lubricant improved by incorporating therein a minor amount, based on the amount of mineral oil, of a halogenated oxygen-bearing organic compound 50 having a vapor pressure less than atmospheric at a temperature of 140° C. 55

5. A lubricating composition containing as a principal lubricating constituent a major amount of mineral lubricating oil with the properties of such composition affecting its use as a lubricant improved by incorporating therein a minor amount, based on the amount of mineral oil, of a halogen and oxygen-bearing organic ring compound. 60

6. A lubricating composition containing as a principal lubricating constituent a major amount of mineral lubricating oil with the properties of such composition affecting its use as a lubricant improved by incorporating therein a minor amount, based on the amount of mineral oil, of a halogen and oxygen-bearing aromatic compound. 70

7. A lubricating composition containing as a principal lubricating constituent a major amount

- of mineral lubricating oil with the properties of such composition affecting its use as a lubricant improved by incorporating therein a minor amount, based on the amount of mineral oil, of a halogen and oxygen-bearing cyclo-aliphatic compound.
8. A lubricating composition containing as a principal lubricating constituent a major amount of mineral lubricating oil with the properties of such composition affecting its use as a lubricant improved by incorporating therein a minor amount, based on the amount of mineral oil, of a halogen and oxygen-bearing hydro-aromatic compound.
15. 9. A lubricating composition containing as a principal lubricating constituent a major amount of mineral lubricating oil with the properties of such composition affecting its use as a lubricant improved by incorporating therein a minor amount, based on the amount of mineral oil, of a halogen and oxygen-bearing alkylated-aromatic compound.
10. 10. A lubricating composition containing as a principal lubricating constituent a major amount of mineral lubricating oil with the properties of such composition affecting its use as a lubricant improved by incorporating therein a minor amount, based on the amount of mineral oil, of a halogen and oxygen-bearing carbon ring compound.
11. A lubricating composition containing as a principal lubricating constituent a major amount of mineral lubricating oil with the properties of such composition affecting its use as a lubricant improved by incorporating therein a minor amount, based on the amount of mineral oil, of a halogen and oxygen-bearing bridged ring compound.
12. A lubricating composition containing as a principal lubricating constituent a major amount of mineral lubricating oil with the properties of such composition affecting its use as a lubricant improved by incorporating therein an effective amount up to 10%, based on the amount of mineral oil, of a halogenated oxygen-bearing organic compound having a vapor pressure less than atmospheric at a temperature of 140° C.
13. A lubricating composition containing as a principal lubricating constituent a major amount of mineral lubricating oil with the properties of such composition affecting its use as a lubricant improved by incorporating therein from about 0.25% to about 2%, based on the amount of mineral oil, of a halogenated oxygen-bearing organic compound having a vapor pressure less than atmospheric at a temperature of 140° C.
14. A lubricating composition containing as a principal lubricating constituent a major amount of mineral lubricating oil with the properties of such composition affecting its use as a lubricant improved by incorporating therein from about 0.25% to about 2%, based on the amount of mineral oil, of a halogen and oxygen-bearing organic ring compound.
15. A lubricating composition containing as a principal lubricating constituent a major amount of mineral lubricating oil with the properties of such composition affecting its use as a lubricant improved by incorporating therein from about 0.25% to about 2%, based on the amount of mineral oil, of a halogen and oxygen-bearing aromatic compound.
16. A lubricating composition containing as a principal lubricating constituent a major amount of mineral lubricating oil with the properties of such composition affecting its use as a lubricant improved by incorporating therein a minor amount, based on the amount of mineral oil, of a halogen and oxygen-bearing organic compound having a vapor pressure less than atmospheric at a temperature of 140° C. and being of the type in which the halogen is directly attached to a ring structure.
17. A lubricating composition containing as a principal lubricating constituent a major amount of mineral lubricating oil with the properties of such composition affecting its use as a lubricant improved by incorporating therein a minor amount, based on the amount of mineral oil, of a halogen and oxygen-bearing organic compound of the type in which the halogen is directly attached to a carbon atom of a benzenoid ring structure.
18. A lubricating composition containing as a principal lubricating constituent a major amount of mineral lubricating oil with the properties of such composition affecting its use as an extreme pressure lubricant improved by incorporating therein a minor amount, based on the amount of mineral oil, of a halogenated oxygen-bearing organic compound having a vapor pressure less than atmospheric at a temperature of 140° C.

CARL F. PRUTTON.  
ALBERT K. SMITH.